

## UNITED STATES PATENT OFFICE

2,042,802

## COLORATION OF MATERIALS

Herbert Platt, Cumberland, Md., assignor to  
Celanese Corporation of America, a corporation  
of Delaware

No Drawing. Application January 26, 1934,  
Serial No. 708,411

20 Claims. (Cl. 8—5)

This invention relates to the dyeing and bottoming of textile yarns and fabrics in which one of the materials employed to impart the color is a so-called natural dye material.

5 An object of the invention is to provide a process whereby materials made from or containing organic derivatives of cellulose may be successfully dyed with natural dyes that are raised to their staple color by chroming.

10 Another object of the invention is to provide a process whereby materials made from or containing organic derivatives of cellulose may be dyed with a bottom color that is a natural chromed dye and then topped with a color that 15 is either a mordant dye, a direct dye, another natural chromed dye, or any other dye having an affinity for the organic derivative of cellulose.

Another object of the invention is to obtain the improved products resulting from this invention. Other objects of this invention will appear from the following detailed description.

Heretofore great difficulty has been experienced in successfully dyeing deep colors on fabrics made of organic esters of cellulose with natural dyes. One of the great sources of annoyance was the production of off shades and unexpected shades.

I have found a process whereby such fibres can be colored to a desired shade successfully and 30 economically by the natural dyes. This makes possible the application of a large class of dye-stuffs to the dyeing of such fibres that heretofore could not be employed with safety. For example, organic derivatives of cellulose may be 35 dyed safely with logwood.

Textile materials dyed according to this invention are not materially weakened nor is there a material change in lustre, hand, or other textile properties.

40 By the method of this invention textile materials may be dyed a thin shade with a natural dye to give a gray or light bottom color that can then be topped up to shade with direct dyeing dyestuffs which is considerably cheaper than attempting to obtain deep colorations free from acid fading by the use of direct dyeing dyestuffs alone. The natural dyes, however, may be employed alone to give deep colors or they may form a deep colored bottom which may be topped 45 with another natural dye to produce the desired shade.

According to this invention, I treat textile materials with a natural dyestuff which is raised to the color desired and made fast by a treatment with a bichromate and an aid such as an

organic acid, a salt of an organic acid or any other aid which is a mild reducing agent.

This invention is applicable to the dyeing of any textile material and especially those made at least in part of organic derivatives of cellulose such as organic esters and ethers of cellulose. Examples of organic esters of cellulose are cellulose acetate, cellulose formate, cellulose propionate and cellulose butyrate, while examples of organic ethers of cellulose are ethyl cellulose, 10 methyl cellulose and benzyl cellulose. Fabrics and yarns which contain mixtures of different types of fibres or filaments may be dyed or cross dyed according to this invention. Thus, yarns and fabrics containing fibres or filaments of 15 organic derivatives of cellulose and wool, or organic derivatives of cellulose and silk, or organic derivatives of cellulose and regenerated cellulose or organic derivatives of cellulose and other fibres or filaments may be dyed according to this 20 invention.

The dyeing may be performed in the yarn, fabric or garment stage of the processing of textiles. Yarn may be dyed as hanks or in packages. The yarn may be woven, warp knitted, 25 circular, knitted or otherwise processed to fabrics and then dyed or such fabrics may be further processed to garments and wearing apparel prior to dyeing.

This invention is applicable to yarns that, if 30 synthetic, may contain incorporated therewith effect materials such as pigments and filling materials, fire retardants, plasticizers, sizes and lubricants. Where, however, such pigments and filling materials as titanium dioxide and antimony 35 trioxide are incorporated with the yarn they have the effect of modifying the resulting color. Thus, when dyeing with logwood, their presence throws the resulting color to the blue side of black in the same dyeing operation that would 40 normally produce a color on the red side of black.

The coloring material may be any of the natural dyes or dye extracts, for example, logwood or haematein, young fustic, fustic, quercitron, Persian berries, weld extract, sandalwood, 45 cutch, etc. The material to be dyed may be placed in a bath about 30 times its own weight of a solution of the natural dye in water. The natural dye may be employed in the solution in 50 from 1 to 10 percent depending upon whether the material is to be dyed as a complete color or dyed as a bottom color. This bath is maintained at 60° to 100° C., preferably about 80° C., and the material is allowed to remain therein for from 20 55

minutes to two hours, depending upon the materials treated and color desired.

The material to be dyed is removed from the natural dye bath and the color top chromed by 5 treating the material containing the natural dye in a bath containing salts of a chromium acid for example sodium or potassium dichromate. This bath may be maintained between 60 and 85° C. depending upon the material treated. For 10 organic derivatives of cellulose being dyed with logwood temperatures of 60° to 100° C., particularly 70° to 80° C. are preferable. The bath may contain from 1 to 4% of the dichromate salt. The bath may also contain aids such as oxalic 15 acid or sodium or potassium oxalate or mixtures of these. It is found that these aids effect some control over the shade of color produced and its fastness to light. Thus, in dyeing with logwood, the presence of an oxalate controls the blueness 20 of the shade and the fastness to light. The percentage of oxalate that may be employed in the bath is between 1 and 3%.

Thus, a good black is obtained on cellulose 25 acetate by dyeing with 10% solution of hæmatein at 80° C. for 1 hour and then chroming with a solution of 2% sodium bichromate and 1.5% sodium oxalate at 75° C. for 30 minutes, rinsing and soaping.

The length of time that dyes, such as logwood, 30 are chromed must be ascertained for each particular fabric material, for when logwood is under-chromed (chromed too little) or over-chromed (chromed too much) lack of light-fastness results; the logwood in the first case turns a reddish brown, whilst in the latter case it turns yellower or greener when exposed to light.

There may be added a small percentage of magnesium sulfate to the dye bath. This salt 35 gives more light fastness to the dye. The presence of various salts also controls the color imparted by such dyes as chromed natural dyestuffs. Thus, in dyeing with a low percentage of logwood as the dyeing material, the presence of magnesium sulphate gives a greyish navy blue, calcium 40 chloride gives a greyish navy blue, calcium hydroxide gives a pearl grey, calcium acetate gives a blue which becomes lighter the greater amount of salt used, while lead acetate gives a greenish to yellowish black.

In dyeing cellulose acetate material with logwood, it is found that using an insufficient 45 amount of sodium bichromate at too low a temperature causes a logwood black that turns a reddish brown on exposure to light, whilst an excessive amount of sodium bichromate at too high a temperature causes a greening of the logwood black. The optimum conditions for a light fast black is a treatment for 20 to 40 minutes with a solution containing 1.5 to 2.5% sodium bichromate maintained at 60-70° C.

The temperature at which logwood is applied 50 has no appreciable effect on the shade or light-resisting properties, except that the higher the temperature, the greater the depth of color obtained.

When fabrics or yarns of subdued lustre, caused 55 either by the presence of finely divided pigments therein or by delustering the same (as by treating cellulose acetate material with hot aqueous soap solutions), are treated by this invention, it is possible to obtain blacks or other dark shades of subdued lustre, whereas bright lustre is obtained by prior methods. Logwood grey or blue 60 may be topped by a second dyeing with logwood

or a direct dye to produce a deep black, while logwood black may be topped by a second dyeing of a natural dye, such as cutch, to give a deep dead black.

According to the method of this invention, the 5 natural dyestuffs readily lend themselves to the printing of fabrics. Thus, organic derivatives of cellulose and silk or mixtures or these may be successfully printed with a paste containing 10 parts of hæmatein, 5 parts of glycerine, 25 parts 10 of glucose, British gum or tragacanth gum, and 60 parts of water. After printing by such means as printing presses, brushing or spraying over stencils and like means, the printed fabric is steamed for about 15 minutes at about 5 lbs. 15 pressure then chromed in a 2% solution of sodium bichromate and 1½% sodium oxalate, or a similar chroming solution after which they are rinsed and soaped. The color imparted is a deep 20 black.

Instead of treating the textile material in a bath of the dye liquor, such dye may be applied to the fabric by padding or other mechanical impregnation, and then fixed either by heating 25 or by batching for a substantial period, after which the fabric may be treated with the chroming bath.

As an aid to the chromate salt in place of oxalic acid or its salts there may be employed any other 30 mild reducing agent, such as ammonium thiocyanate or alkali sulphites. The ammonium sulphocyanide may be used alone or in connection with the oxalic acid or its salts. These materials effect both the trueness of color and its fastness 35 to light.

As a means of further describing the invention there are given the following examples.

#### Example I

Cellulose acetate fabric is dyed by treating for 40 1 hour with a ½% solution of logwood crystals at 80° C., and then chromed with a 2% solution of sodium bichromate having 1½% of sodium oxalate therein. The chrome bath is maintained at 45 60° and the treatment is for 30 minutes.

A blue grey shade is obtained. This grey may be used as such or used as a bottom color to be topped with a direct dye, another logwood dyeing or another natural dye.

#### Example II

The material dyed or bottomed by Example I is topped with a mixture of direct dyes of yellow, orange and red colors. The shade is thus brought 55 up to a dead black.

#### Example III

A material woven of natural silk and cellulose acetate containing titanium oxide is dyed for one 60 hour at 80° C. in a 30:1 bath. This bath contained 3% logwood crystals and 0.25% cutch.

This material is then chromed in a bath containing 2% sodium bichromate and 1½% sodium oxalate.

The color imparted is a black slightly to the green side of black.

#### Example IV

A material of cellulose acetate is dyed with a 70 solution of 10% logwood for 1 hour at 80° C., rinsed, and treated with 2% sodium bichromate and 1½% sodium oxalate solution for 30 minutes at 70-75° C., rinsed and soap scoured.

The material thus treated is of a deep black color and is heavily delustered.

As a guide to the range of shades obtainable from various percentages of logwood reference 5 may be had to the following table.

Woven fabric of cellulose acetate is dyed in various concentrations of logwood crystals for one hour at 80° C. in a 30:1 bath, chromed with sodium bichromate at 60° C. for 30 minutes, weaker solutions of the alkali bichromate being used for the weaker concentration of logwood.

|    | Percent solution of log-wood | Percent solution Na <sub>2</sub> Cr <sub>2</sub> O <sub>7</sub> and an aid | Shade obtained      |
|----|------------------------------|----------------------------------------------------------------------------|---------------------|
| 15 | 0.1                          | 1.0                                                                        | Light neutral grey. |
|    | 0.2                          | 1.0                                                                        | Pale grey.          |
|    | 0.25                         | 1.0                                                                        | Slate grey.         |
| 20 | 0.50                         | 1.0                                                                        | Dark grey.          |
|    | 0.75                         | 1.0                                                                        | Do.                 |
|    | 1.0                          | 1.0                                                                        | Dark greyish blue.  |
|    | 1.25                         | 2.0                                                                        | Dark greyish black. |
|    | 1.50                         | 2.0                                                                        | Do.                 |
|    | 1.75                         | 2.0                                                                        | Yellowish black.    |
|    | 2.0                          | 2.0                                                                        | Black.              |
| 25 | 3                            | 2                                                                          | Deep black.         |

There is apparently no difference as to which of the alkali metal salts of either the chromic acid or oxalic acid are employed.

Having described the invention, what I desire to secure by Letters Patent is:

1. The process of imparting color to textile materials which comprises applying thereto a natural mordant dyestuff requiring an after treatment with a salt of a chromic acid, an alkali salt of a chromic acid and a compound selected from the group consisting of oxalic acid, alkali salts of oxalic acid, ammonium thiocyanate and alkali sulphites.

2. The process of imparting color to textile materials comprising organic derivatives of cellulose which comprises applying thereto a natural mordant dyestuff requiring an after-treatment with a salt of a chromic acid, an alkali salt of a chromic acid and a compound selected from the group consisting of oxalic acid, alkali salts of oxalic acid, ammonium thiocyanate and alkali sulphites.

3. The process of imparting color to textile materials comprising cellulose acetate which comprises applying thereto a natural mordant dyestuff requiring an after-treatment with a salt of a chromic acid, an alkali salt of a chromic acid and a compound selected from the group consisting of oxalic acid, alkali salts of oxalic acid, ammonium thiocyanate and alkali sulphites.

4. The process of imparting color to textile materials comprising synthetic filaments of a cellulose derivative containing finely divided pigments therein which comprises applying thereto a natural mordant dyestuff requiring an after-treatment with a salt of a chromic acid, a chromic acid alkali salt and a compound selected from the group consisting of oxalic acid, alkali salts of oxalic acid, ammonium thiocyanate and the alkali sulphite salts.

5. The process of imparting color to textile materials comprising filaments of cellulose acetate containing finely divided pigments therein which comprises applying thereto a natural mordant dyestuff requiring an after treatment with a salt of a chromic acid, an alkali salt of chromic acid and a compound selected from the group consisting of oxalic acid, alkali salts of oxalic acid, ammonium thiocyanate and the alkali sulphite salts.

6. The process of imparting color to textile ma-

terials which comprises applying thereto a natural mordant dyestuff requiring an after-treatment with a salt of a chromic acid and chroming same with an alkali dichromate in the presence of an alkali oxalate.

5

7. The process of imparting color to textile materials comprising organic derivatives of cellulose which comprises applying thereto a natural mordant dyestuff requiring an after-treatment with a salt of a chromic acid and chroming same with an alkali dichromate in the presence of an alkali oxalate.

10

8. The process of imparting color to textile materials comprising cellulose acetate which comprises applying thereto a natural mordant dye- 15 stuff requiring an after-treatment with a salt of a chromic acid and chroming same with an alkali dichromate in the presence of an alkali oxalate.

15

9. The process of imparting color to textile materials comprising organic derivatives of cellulose 20 which comprises applying thereto a bottoming color of a natural mordant dyestuff requiring an after-treatment with a salt of a chromic acid, chroming same with an alkali dichromate in the presence of alkali oxalate and then applying a 25 topping color.

25

10. The process of imparting color to textile materials comprising cellulose acetate which comprises applying thereto a bottoming color of a natural mordant dyestuff requiring an after-treatment with a salt of a chromic acid, chroming same with an alkali dichromate 30 in the presence of alkali oxalate and then applying a topping color.

30

11. The process of imparting color to textile 35 materials comprising organic derivatives of cellulose which comprises applying thereto a bottoming color of a natural mordant dyestuff requiring an after-treatment with a salt of a chromic acid, chroming same with an alkali dichromate 40 in the presence of an alkali oxalate and then applying a natural dye as a topping color and chroming same.

35

12. The process of imparting color to textile 45 materials comprising cellulose acetate which comprises applying thereto a bottoming color of a natural mordant dyestuff requiring an after-treatment with a salt of a chromic acid, chroming same with an alkali dichromate in the presence of an alkali oxalate and then applying a natural 50 dye as a topping color and chroming same.

45

13. The process of imparting deep colorations to textile materials while retaining a subdued lustre comprising applying to textile materials of subdued lustre comprising derivatives of cellulose 55 a logwood dye, chroming same with a chromate in the presence of a substance selected from the group consisting of oxalic acid, alkali salts of oxalic acid, ammonium thiocyanate and alkali sulphite.

55

14. The process of imparting deep colorations to textile materials while retaining a subdued lustre comprising applying to textile materials of subdued lustre comprising cellulose acetate a logwood dye, chroming same with a chromate in the 65 presence of a substance selected from the group consisting of oxalic acid, alkali salts of oxalic acid, ammonium thiocyanate and alkali sulphite.

60

15. The process of imparting color to textile materials which comprises applying thereto log- 70 wood from an aqueous bath and chroming the log-wood treated textile materials with an aqueous bath containing an alkali dichromate and an alkali oxalate.

70

16. The process of imparting color to textile 75

materials comprising organic derivatives of cellulose which comprises applying thereto logwood from an aqueous bath and chroming the logwood treated textile materials with an aqueous bath containing an alkali dichromate and an alkali oxalate.

17. The method of imparting color to textile materials which comprises printing the material with a paste comprising a natural mordant dye-  
10 stuff requiring an after-treatment with a salt of a chromic acid, steaming the printed textile material and chroming in a solution comprising an alkali dichromate and an alkali oxalate.

18. A textile material colored with a natural mordant dyestuff requiring an after-treatment

with a salt of a chromic acid chromed with a solution containing an alkali dichromate and an alkali oxalate.

19. A textile material colored with a natural mordant dyestuff requiring an after-treatment 5 with a salt of a chromic acid chromed with a solution containing an alkali dichromate and a compound selected from the group consisting of oxalic acid, alkali salts of oxalic acid, ammonium thiocyanate and alkali sulphite salts.

20. A textile material colored with logwood chromed with an alkali dichromate and an alkali oxalate.

HERBERT PLATT.